# EUROPEAN PATENT SPECIFICATION

(11) **EP 3 838 443 B1**
(45) Date of publication and mention of the grant of the patent: **29.05.2024**
(21) Application number: 19850707.1
(22) Date of filing: 13.08.2019
(51) Int. Cl.: B22F 3/10, B22F 3/16, B22F 3/00, B22F 3/02

(54) **A FRICTION MATERIAL MANUFACTURING APPARATUS AND METHOD**
VORRICHTUNG UND VERFAHREN ZUR HERSTELLUNG VON REIBUNGSMATERIAL
DISPOSITIF ET PROCÉDÉ DE PRODUCTION DE MATÉRIAU DE FRICTION

(30) Priority: 13.08.2018 JP 2018152363; 17.07.2019 JP 2019132171
(43) Date of publication of application: 23.06.2021
(73) Proprietor: Akebono Brake Industry Co., Ltd., Tokyo 103-8534 (JP)
(72) Inventor: KATO, Masanori, Tokyo 103-8534 (JP); TAKAHASHI, Hideaki, Tokyo 103-8534 (JP); ONODERA, Katsuhiro, Tokyo 103-8534 (JP); NIHEI, Marina, Tokyo 103-8534 (JP); UENO, Atsushi, Tokyo 103-8534 (JP); TAKADA, Eri, Tokyo 103-8534 (JP)
(74) Representative: Grünecker Patent- und Rechtsanwälte PartG mbB
(86) International application number: PCT/JP2019/031836
(87) International publication number: WO 2020/036176

(56) References cited:
- CN-U- 205 437 147
- JP-A- H0 331 689
- JP-A- S5 265 703
- JP-A- S5 265 703
- JP-A- 2016 141 847
- US-A1- 2017 182 683

## Description

### TECHNICAL FIELD

The present application discloses a friction material manufacturing apparatus and a friction material manufacturing method.

### BACKGROUND ART

Brakes used in vehicles and other various machines are usually provided with friction materials. The friction material is a member that converts kinetic energy into thermal energy, and thus is required to exert a predetermined braking force even at a high temperature. Therefore, in order to exert the predetermined braking force even when the friction material is used in a high-temperature state, various measures for shaping the friction material at an appropriate temperature are made in a manufacturing line of the friction material (see Patent Literatures 1 to 3).

Further relevant prior art is described in US 2017/182683 A1, JP S52 65703 A, CN 205 437 147 U and JP 2016 141847 A

### CITATION LIST

### PATENT LITERATURE

Patent Literature 1: JP-A-2016-522362
Patent Literature 2: Japanese Patent No. 6113927
Patent Literature 3: Chinese Utility Model No. 205437147

### SUMMARY OF INVENTION

### TECHNICAL PROBLEM

For example, in order to efficiently manufacture a friction material having a relatively high temperature during molding as typified by a friction material obtained by sintering a metal powder, it is desired to rapidly heat the friction material. However, when the temperature of the friction material is raised by a hot plate, heat is transferred from a heat source to the friction material via the hot plate, and thus a temperature rise rate of the friction material greatly depends on a heat capacity of the hot plate in accordance with temperature rise of the heat plate per se. Further, when the temperature of the friction material is raised in a convection oven, heat is transferred from the heat source to the friction material via a gas flow, and thus it is difficult to quickly raise the temperature of the friction material via the gas, which has poor heat transfer property.

An object of the present invention is to enable efficient manufacture of a friction material.

### SOLUTION TO PROBLEM

In particular in order to solve the aforementioned problem, it is provided a friction material manufacturing apparatus which is having the features as defined in defined in claim 1. Further, it is provided the friction material manufacture method, which has the features defined in claim 12. Further preferred embodiments are defined in the dependent claims.

More specifically, the present invention is a friction material manufacturing apparatus configured to sinter friction materials, and includes: a jig configured to clamp a stack of workpieces, which are preforms of the friction materials, in a stacking direction; a transport mechanism that forms a transport path of the jig; and a heating apparatus provided in a way of the transport path and configured to heat the stack clamped by the jig with infrared rays from a lateral side with respect to the stacking direction.

The friction material manufacturing apparatus described above uses infrared rays to heat the stack clamped by the jig, and thus is capable of heating a portion of the stack in a selectively concentrated manner. Therefore, for example, the heating target can be efficiently heated as compared with a heating method that is difficult to heat a specific place in a selectively concentrated manner, such as in a convection method.

Since the friction material manufacturing apparatus described above has an aspect in which the heating apparatus is provided in a way of the transport path and the jig for clamping the stack to be heated is transported by the transport mechanism, the stack that has been heated by the heating apparatus can be separated integrally with the jig from the heating apparatus. Therefore, while waiting for a decrease in the temperature of the stack that has been heated by the heating apparatus, a stack clamped by another jig can be continuously heated by the heating apparatus.

Therefore, according to the friction material manufacturing apparatus described above, it is possible to efficiently manufacture friction materials.

The jig may include: a support portion configured to support the stack from one side in the stacking direction; and a pressing portion configured to press the stack from the other side in the stacking direction toward the support portion. By using such a jig, the stack that has been heated by the heating apparatus can be separated from the heating apparatus integrally with the jig from the heating apparatus while maintaining a pressed state. For this reason it is possible to quickly replace the stack to be heated in the heating apparatus.

The heating apparatus may include an element configured to emit infrared rays at a position that is on the lateral side of the stack in a state where the jig is at a position of the heating apparatus. In the heating apparatus having the element configured to emit infrared rays at such a position, the stack clamped by the jig can be irradiated by the infrared rays of the element only by simply conveying the jig clamping the stack to be heated to the vicinity of the heating apparatus by the transport mechanism, and thus it is possible to quickly replace the stack to be heated in the heating apparatus.

The jig may include a window made from a transparent plate configured to cover the stack from the lateral side with respect to the stacking direction, and may include an accommodation portion configured to accommodate the stack. In this case, the jig may include a gas introduction portion configured to introduce an inert gas into the accommodation portion. The friction material manufacturing apparatus described above uses infrared rays for heating, and thus is capable of heating through such window made from a transparent plate. Therefore, by adopting such configuration in which the accommodation portion is provided in the jig and heating by infrared rays is performed through the window made from a transparent plate, for example, the inside of the accommodation portion can be applied with an inert gas atmosphere.

The friction material manufacturing apparatus may further include an accommodation portion configured to accommodate the jig, the transport mechanism, and the heating apparatus. The accommodation portion may include a gas introduction portion configured to introduce an inert gas. In this case, for example, even if the inside of the accommodation portion is applied with an inert gas atmosphere, the jig can be easily moved.

In addition, the friction material manufacturing apparatus may further include an accommodation portion configured to accommodate the heating apparatus, and allow the jig to move in and out. The accommodation portion may include a door at an opening portion through which the jig is to move in and out. In this case, the accommodation portion may include an introduction portion configured to introduce an inert gas. By providing the accommodation portion in the heating apparatus in this manner and closing the accommodation portion after the jig is transported to the vicinity of the heating apparatus by the transport mechanism, the inside of the accommodation portion can be applied with an inert gas atmosphere.

The jig may include a heat insulating member at a portion to be in contact with the stack. In this case, heat transfer from the stack to the jig can be prevented.

The heating apparatus may be a near infrared heater having a peak wavelength in a range of 1200 nm to 1700 nm. The near infrared ray having such a wavelength is higher in permeability in substance than, for example, in mid-infrared rays having a peak wavelength of 1700 nm to 2700 nm, and thus is capable of heating the inside of the stack with high energy without remaining in the vicinity of the surface even with respect to a stack obtained by stacking friction materials. Therefore, it is suitable for heating a heating object that whose center portion cannot be easily heated, such as a stack obtained by stacking friction materials.

The invention can also be understood from an aspect of method. For example, the present invention may be a friction material manufacturing method for sintering friction materials, the friction material manufacturing method including: clamping, by a jig, a stack of workpieces, which are preforms of the friction materials, in a stacking direction; transporting the jig along a transport path formed by a transport mechanism; and heating, by a heating apparatus provided in a way of the transport path, the stack clamped by the jig with infrared rays from a lateral side with respect to the stacking direction.

### ADVANTAGEOUS EFFECTS OF INVENTION

The present invention enables efficient manufacture of a friction material.

### BRIEF DESCRIPTION OF DRAWINGS

[Fig. 1] Fig. 1 is a schematic configuration diagram of a friction material manufacturing apparatus according to an embodiment.
[Fig. 2] Fig. 2 is a structural view of the friction material manufacturing apparatus as viewed from a lateral side of a transport path.
[Fig. 3] Fig. 3 is a structural view of the friction material manufacturing apparatus as viewed from a transport direction of the transport path.
[Fig. 4] Fig. 4 is a first diagram illustrating a method for using the friction material manufacturing apparatus.
[Fig. 5] Fig. 5 is a second diagram illustrating a method for using the friction material manufacturing apparatus.
[Fig. 6] Fig. 6 is a diagram showing a state where jigs are arranged continuously.
[Fig. 7] Fig. 7 is a diagram showing a modification of the friction material manufacturing apparatus.
[Fig. 8] Fig. 8 is a diagram illustrating an example of openings for gas provided on an upper plate and a lower plate.
[Fig. 9] Fig. 9 is a diagram showing a first modification of the friction material manufacturing apparatus.
[Fig. 10] Fig. 10 is a structural view of the friction material manufacturing apparatus according to the first modification as viewed from a lateral side of the transport path.
[Fig. 11] Fig. 11 is a diagram showing a second modification of the friction material manufacturing apparatus.
[Fig. 12] Fig. 12 is a diagram showing a third modification of the friction material manufacturing apparatus.
[Fig. 13] Fig. 13 is a diagram showing a fourth modification of the friction material manufacturing apparatus.

### DESCRIPTION OF EMBODIMENTS

Fig. 1 is a schematic configuration diagram of a friction material manufacturing apparatus according to an embodiment. A friction material manufacturing apparatus 1 is an apparatus for sintering friction materials for brakes, and includes: a jig 4 for clamping in a stacking direction, with a pressing mechanism 3, a stack 2 obtained by stacking workpieces, which are preforms of the friction materials; a transport mechanism that forms a transport path 5 of the jig 4; and a heating apparatus 6 provided in a way of the transport path 5 for heating the stack 2 clamped in the pressing mechanism 3 by the jig 4 with infrared rays from a lateral side with respect to the stacking direction. The friction material manufacturing apparatus 1 moves the jig 4 in a state where the stack 2 is clamped by the pressing mechanism 3 along the transport path 5, and heats the friction materials in the stack 2 by heating the stack 2 with the heating apparatus 6 in a way of the transport path 5. The friction material manufacturing apparatus 1 is not limited to a structure in which the stack 2 is clamped vertically, and may have a structure in which the stack 2 is clamped horizontally. The friction material is assumed to be used in, for example, various industrial equipment, transportation equipment, office equipment, or the like.

The stack 2 is obtained by stacking, on a pressure plate, preforms each obtained by mixing a metal powder with an abrasive and/or a lubricant and pressing it into a thin plate shape, and further stacking a plurality of groups of assemblies each obtained by arranging an alumina setter on a friction surface side of the preform. The stack 2 can be realized by setting and stacking the preform, the pressure plate, and the setter on, for example, a jig for stacking.

The jig 4 includes an accommodation portion 7 capable of accommodating the stack 2 in a state of being clamped by the pressing mechanism 3. The accommodation portion 7 is provided with a window through which near infrared rays of the heating apparatus 6 pass, as will be described later. The accommodation portion 7 is formed of a material having heat resistance to the heat of the heating apparatus 6.

The components of the friction material manufacturing apparatus 1 will be described in detail. Fig. 2 is a structural view of the friction material manufacturing apparatus 1 as viewed from a lateral side of the transport path 5. Fig. 3 is a structural view of the friction material manufacturing apparatus 1 as viewed from a transport direction of the transport path 5.

The friction material manufacturing apparatus 1 includes a transport mechanism 8 that forms the transport path 5 and a support member 9 that supports the heating apparatus 6. An inert gas cylinder 10 is provided together with the friction material manufacturing apparatus 1, and the inert gas cylinder 10 is connected to a gas introduction port 12 of the jig 4 via a hose 11. The inert gas supplied from the inert gas cylinder 10 flows into the accommodation portion 7 of the jig 4. Examples of the inert gas filled in the inert gas cylinder 10 include argon gas, nitrogen gas, and various other inert gases. The inert gas cylinder 10 is provided for the purpose of preventing oxidation during sintering by applying an inert gas atmosphere inside the accommodation portion 7 in which the stack 2 is accommodated. In addition to the inert gas atmosphere, sintering may also be performed in a reducing gas atmosphere, in a combination atmosphere of an inert gas and a reducing gas, or in a reduced pressure atmosphere. Therefore, the hose 11 connecting the inert gas cylinder 10 and the gas introduction port 12 of the jig 4 is routed such that the jig 4 can be traced even when sliding along the transport path 5.

The accommodation portion 7 is provided with a quartz glass 13 through which the near infrared rays of the heating apparatus 6 are transmitted. The accommodation portion 7 is basically formed of a metal material having heat resistance to heat of the heating apparatus 6, such as stainless steel, and is designed such that the quartz glass 13 is disposed at a portion irradiated by the near infrared rays of the heating apparatus 6 when the jig 4 is in the vicinity of the heating apparatus 6, and the near infrared rays of the heating apparatus 6 are unlikely to be irradiated onto unnecessary portions of the jig 4. In the quartz glass 13 and the other parts of the accommodation portion 7 formed of the metal material, each member is designed to have an appropriate size so that leakage of the inert gas flowing inside falls within a predetermined allowable range and expansion of the members caused by temperature rise by the heating apparatus 6 does not cause interference between the members. The inert gas of the inert gas cylinder 10 introduced into the accommodation portion 7 through the gas introduction port 12 passes through the accommodation portion 7 and is exhausted through a gas exhaust port 17 provided in the accommodation portion 7. The inert gas introduced into the accommodation portion 7 through the gas introduction port 12 prevents oxidation of the friction material, and exerts a cooling function of the members constituting the accommodation portion 7 and a contamination preventing function of the quartz glass 13, and thus an exhaust amount through the gas exhaust port 17 is adjusted in consideration of maintaining these functions. The transparent plate window covering the stack 2 from the lateral side with respect to the stacking direction is not limited to the quartz glass 13 as long as transmitting infrared light and having heat resistance.

The pressing mechanism 3 provided in the accommodation portion 7 includes a support portion 14 that supports the stack 2 from above, and a pressing portion 15 that presses the stack 2 from below toward the support portion 14. The pressing portion 15 is a part raised and lowered vertically by an air cylinder 16. The air cylinder 16 is connected to a compressor that supplies high-pressure air via a pressure-resistant hose, and raises and lowers the pressing portion 15 in accordance with opening and closing of a valve provided in a way of a path for supplying the high-pressure air. In addition, a load cell for measuring a load applied to the stack 2 is provided in the pressing mechanism 3, and the magnitude of the load applied to the stack 2 can be adjusted. The pressing mechanism 3 is provided with a cooling structure such as a water-cooling jacket for preventing damage to the load cell due to the heat of the heating apparatus 6. The pressing mechanism 3 is only required to be able to press the stack 2, and may be, other than the air cylinder 16, for example, a coil spring, a lever in combination with a weight, a manual jack, a hydraulic cylinder, or various other pressing means.

The jig 4 configured as described above can be slid along the transport path 5 by the transport mechanism 8. The transport mechanism 8 for sliding the jig 4 may be a roller-type conveyor on which the jig 4 is placed, or may be a linear guide that is fitted to a rail extending along the transport path 5. The transport mechanism 8 may be a manual mechanism without a power source that slides the jig 4, such as a motor, or may be an automatic mechanism including a power source.

The jig 4 is transported on the transport path 5 while being advanced or stopped at an appropriate timing. The timing at which the jig 4 is advanced or stopped is determined according to a heating capacity of the heating apparatus 6, an atmosphere temperature in a plant in which the friction material manufacturing apparatus 1 is provided, a composition of the friction materials stacked in the stack 2, the number of friction materials stacked in the stack 2, the pressing force of the pressing mechanism 3, and other various factors.

The heating apparatus 6 heats the stack 2 set in such a jig 4 by near infrared rays. The heating apparatus 6 includes a plurality of rod-shaped near infrared heaters extending along the direction of the transport path 5 on both sides thereof, and has a heating capacity capable of heating the stack 2 to about 1000°C.

Each near infrared heater emits, for example, near infrared rays having a peak wavelength in a range of 1200 nm to 1700 nm. The near-infrared ray having such a wavelength is higher in permeability in substance than in far infrared rays, and thus is capable of heating the inside of the stack 2 without remaining in the vicinity of the surface even with respect to the stack 2 obtained by stacking friction materials. Therefore, it is suitable for heating the stack 2 with infrared rays through the quartz glass 13.

In the near infrared heaters, energization is controlled for each combination of one to a plurality of the heats, and an appropriate amount of heat can be applied to each of an upper layer portion, a middle layer portion, and a lower layer portion of the stack 2. The energization pattern of each near infrared heater of the heating apparatus 6 is adjusted according to the heating capacity of the heating apparatus 6, the atmosphere temperature in a plant in which the friction material manufacturing apparatus 1 is provided, the composition of the friction materials stacked in the stack 2, the number of friction materials stacked in the stack 2, the pressing force of the pressing mechanism 3, and other various factors. The energization pattern of the heating apparatus 6 may be in accordance with a predetermined sequence set in advance, or in accordance with information of a radiation thermometer for measuring the temperature of the stack 2 in a non-contact manner, such as thermography.

Next, a method for using the friction material manufacturing apparatus 1 will be described. Fig. 4 is a first diagram illustrating a method for using the friction material manufacturing apparatus 1. Fig. 5 is a second diagram illustrating a method for using the friction material manufacturing apparatus 1. When the friction material is sintered using the friction material manufacturing apparatus 1, first, as shown in (A) of Fig. 4, the air cylinder 16 is contracted to bring the pressing portion 15 to a lower limit position, and the stack 2 is set in the jig 4 in this state. Next, as shown in (B) of Fig. 4, the air cylinder 16 is extended to raise the pressure portion 15, and the stack 2 is clamped between the support portion 14 and the pressing portion 15. Then, an open portion of the accommodation portion 7 is closed, and the inert gas of the inert gas cylinder 10 is supplied into the accommodation portion 7.

When the heating apparatus 6 is ready for heating in this manner, as shown in (C) of Fig. 4, the jig 4 is slid by the transport mechanism 8, and the jig 4 is moved to the vicinity of the heating apparatus 6. Then, the stack 2 is heated by the heating apparatus 6. When sintering of the friction materials stacked in the stack 2 proceeds, the jig 4 is slid at an appropriate timing to separate the jig 4 from the heating apparatus 6 as shown in (A) of Fig. 5. Then, when the stack 2 is cooled by natural cooling or the like until the friction materials stacked in the stack 2 are cooled to an appropriate temperature, sintering of the friction materials stacked in the stack 2 is completed. When sintering of the friction materials stacked in the stack 2 is completed, as shown in (B) of Fig. 5, the air cylinder 16 is contracted to bring the pressing portion 15 to the lower limit position, and the stack 2 is removed from the jig 4 in this state. The jig 4 from which the stack 2 is removed can be immediately used for sintering other friction materials.

The near infrared heaters have a temperature rise rate of 10 times to 20 times as compared with a resistance heater. In addition, the near infrared heaters have a peak wavelength shorter than in the range of 1700 nm to 2700 nm, which is the peak wavelength of medium-wavelength carbon heater or medium-wavelength infrared heater, and thus can output higher energy than the medium-wavelength carbon heater or medium-wavelength infrared heater, and can sinter a friction material of an inorganic substance obtained by mixing an abrasive and/or a lubricant into a metal powder in a relatively short time.

In the friction material manufacturing apparatus 1 of the embodiment described above, since the jig 4 in which the stack 2 is set can pass through the vicinity of the heating apparatus 6 while being slid by the transport mechanism 8, for example, the friction materials can be fired in a large amount in a substantially continuous manner instead of a batch manner by being used as described below.

Fig. 6 is a diagram showing a state where jigs 4 are arranged continuously. In the friction material manufacturing apparatus 1, since each jig 4 in which the stack 2 is set can pass through the vicinity of the heating apparatus 6 while being slid by the transport mechanism 8, for example, as shown in Fig. 6, by providing the plurality of jigs 4 (4-1 to 5) in which the stack 2 is set in the transport path 5, a jig 4 whose heating of the stack 2 is completed in the heating apparatus 6 can be moved away from the heating apparatus 6, and a subsequent jig 4 in which a stack 2 before heating is set can be continuously slid and placed at the position of the heating apparatus 6, whereby heating and cooling of the friction materials can be performed at the same time. Therefore, it is possible to increase the use efficiency of the heating apparatus 6 as much as possible. Since the friction material manufacturing apparatus 1 can be used in this manner, a region where the heating apparatus 6 is present in the transport path 5 can be regarded as a heating zone and a region other than the heating zone can be regarded as a cooling zone.

In the friction material manufacturing apparatus 1 of the above embodiment, sintering of the friction materials is performed only by the heating apparatus 6, but the sintering of the friction materials may also be performed in cooperation of the heating apparatus 6 and another heating apparatus. For example, a convection oven using hot air may be provided next to the heating apparatus 6 including the near infrared heaters together with the friction material manufacturing apparatus 1, so that the heating apparatus 6 raises the temperature of the friction materials, and the convection oven maintains the temperature of the friction materials heated by the heating apparatus 6. The temperature of the friction materials may be maintained by independently changing outputs of the plurality of near infrared heaters of the heating apparatus 6.

Fig. 7 is a diagram showing a modification of the friction material manufacturing apparatus 1. For example, as shown in Fig. 7, the friction material manufacturing apparatus 1 may be an apparatus in which a plurality of heating apparatuses 6 are provided along the transport path 5. If the friction material manufacturing apparatus 1 is provided with a plurality of heating apparatuses 6 along the transport path 5, the respective stacks 2 set in the plurality of jigs 4 can be simultaneously heated by the plurality of heating apparatuses 6. Therefore, the friction material manufacturing apparatus 1 of the present modification can sinter a large number of friction materials.

A case of producing sintered friction materials using near infrared heaters and a case of producing sintered friction materials using resistance heaters were compared and verified, and the results are shown below. In this verification, the stack 2 was placed such that the stacking direction of the stack 2 was horizontal instead of vertical as in the embodiment described above, and the stack 2 was heated from the upper side and the lower side.

In the present verification, the rod-shaped near infrared heaters constituting the heating apparatus have a peak wavelength of 1200 nm to 1700 nm, a total length of 405 mm, and a length of heating portion (effective length) of 340 mm. In this verification, six near infrared heaters were arranged on the upper side, and three were arranged on the lower side of the stack 2 arranged to have the horizontal stacking direction.

In the present verification, a jig corresponding to the jig 4 of the above embodiment was prepared by forming a pressing mechanism with a coil spring, and introducing an argon gas into a sealed accommodation portion formed from a heat-resistant metal component and a transparent quartz glass. Since the effective length of the near infrared heaters is 340 mm, by setting a frame of the jig to a length of about 540 mm, the metal component constituting the frame of the jig is unlikely to be directly irradiated by near infrared rays emitted from the near infrared heaters.

In this verification, argon gas was introduced into the accommodation portion through the introduction port of two systems, and discharged from the exhaust port of one system. Further, when the argon gas flows from the introduction port of the two systems into the accommodation portion, the argon gas was constantly cooled by being blown to the coil spring constituting the pressing mechanism, thereby preventing thermal deformation of the coil spring.

In this verification, a metal powder was mixed with an abrasive and a lubricant and pressed into a thin plate, so as to prepare six preforms of a cylindrical block having a diameter of 42 mm and a thickness of 12 mm. Then, the cylindrical blocks were stacked on a hot rolled steel plate corresponding to the pressure plate of the brake, and alumina was further interposed therebetween to form a stack. The stack was heated in a state applied with a load of 3.0 MPa by the coil spring. Heights of the upper and lower near infrared heaters were adjusted such that a distance between centers of the near infrared heaters and centers of the cylindrical blocks was 70 mm. Argon gas was continuously flowed into the accommodation portion at a pressure of 0.45 MPa. Gas replacement (purge) in the accommodation portion was 5 minutes.

The near infrared heaters were controlled such that a full output of the upper and lower heaters was 20 kW, and an output ratio of the upper to the lower heaters was 16.8 to 4.9. Then, after a temperature of a thermocouple attached to the stack to be heated reached 950°C, the temperature was maintained at 950 ± 15°C for 30 minutes, and then the energization of the near infrared heaters was turned off. In addition, the introduction of argon gas was continued until the stack to be heated reached normal temperature.

The sintered friction materials produced by the method corresponding to the above embodiment are hereinafter referred to as examples. The evaluation results of comparison between the examples and comparative examples prepared with a sintering furnace using resistance heaters will be described below. The comparative examples were prepared in an argon gas atmosphere at a surface pressure of 3.0 MPa, a sintering temperature of 950°C, a maintaining time of 30 minutes, and a heating rate of 10°C / min.

In this evaluation, the following five items were evaluated.
1. Time until the sintering temperature reaches 950°C
2. Shrinkage factor
3. Surface hardness
4. Base material shear strength
5. Pressure plate (PP) adhesive shear strength

The evaluation results of the items are shown in the following table.

**[Table 1]**

| Heated samples | Examples | Comparative examples |
|---|---|---|
| Heating method | Near infrared heater | Resistance heater |
| Time until reaching 950°C (min) | 7.2 | 95 |
| Shrinkage factor (%) | 7.7 (6.7 to 8.3) | 8.9 (8.4 to 9.3) |
| Surface hardness (HRS) | 48 (30 to 58) | 50 (46 to 53) |
| Base material shear strength (MPa) | 3.6 (2.9 to 4.5) | 2.5 (2.2 to 2.6) |
| PP adhesive shear strength (MPa) | 30.7 (27.6 to 33.8) | 19.1 (18.3 to 20.0) |

| | | |
|---|---|---|
| * The numbers are average values, and the numbers in the parentheses indicate minimum values and maximum values. | | |

As can be seen from the table above, in the case of the examples, the sintering temperature reached 950°C in an extremely short time of about 1/10 as compared with the case of the comparative examples. In addition, the shrinkage factor and the surface hardness were similar in the examples and the comparative examples. Regarding the base material shear strength and the PP adhesive shear strength, the examples had a tendency to be 1.4 times to 1.6 times higher than that of the comparative examples.

From the above results, it was confirmed that the examples were capable of producing sintered friction materials having performances similar as that of the comparative examples in a temperature rise time of about 90 minutes shorter than the comparative examples. In this verification, the sintering temperature was set to 950 ± 15°C, the sintering retention time was set to 30 minutes, and the sintering surface pressure was set to 3.0 MPa, whereas the sintering temperature in the sintering process is preferably 900°C to 1300°C, more preferably 950°C to 1250°C. The sintering retention time is preferably 30 minutes to 180 minutes. The sintering surface pressure is preferably 1 MPa to 18 MPa. As long as the sintering temperature, the sintering retention time, and the sintering surface pressure are within these ranges, the same effect as in the above examples is exhibited.

Although manufacturing of sintered friction materials is assumed in the above description, the friction material manufacturing apparatus 1 of the above embodiment can be used not only for manufacturing of sintered friction materials, but also for manufacturing of resin-based friction materials containing a large amount of organic materials, for example.

A lower plate constituting a bottom surface and an upper plate constituting a top surface of the accommodation portion 7 may be configured as follows. Fig. 8 is a diagram illustrating an example of openings for gas provided on the upper plate and the lower plate. The accommodation portion 7 may be formed from, for example, a lower plate having five gas introduction ports LF1 to LF5 arranged side by side on a front side and five gas introduction ports LB1 to LB5 arranged side by side on a back side of the friction material manufacturing apparatus 1, and an upper plate having five gas exhaust ports UF1 to UF5 arranged side by side on the front side and five gas exhaust ports UB1 to UB5 arranged side by side on the back side of the friction material manufacturing apparatus 1. In this case, the lower plate is provided with a first internal flow path for supplying the gas to the gas introduction ports LF1 to LF5, and a second internal flow path for supplying the gas to the gas introduction ports LB1 to LB5.

If the accommodation portion 7 includes such upper plate and lower plate, the gas blown from the gas introduction ports LF1 to LF5, LB1 to LB5 flows along the surface of the quartz glass 13, and is discharged from the gas exhaust ports UF1 to UF5, UB1 to UB5. Therefore, the surface of the quartz glass 13 is prevented from contamination by the gas. Although Fig. 8 shows a state where ten gas openings are provided in each of the upper plate and the lower plate, the diameters and the numbers of the gas introduction ports LF1 to LF5, LB1 to LB5, the diameters and the numbers of the gas exhaust ports UF1 to UF5, UB1 to UB5, and a flow rate of the gas can be appropriately set according to a size, a shape, a heating temperature, and the like of the workpieces. Further, unnecessary openings may be closed with a plug, for example corresponding to, the size, shape, heating temperature, and the like of the workpieces.

In addition, the support portion 14 that supports the stack 2 obtained by stacking the workpieces from above and/or the pressing portion 15 that presses the stack 2 from below toward the support portion 14 may include a heat insulating member at a portion in contact with the stack 2. If a heat insulating member is provided at the portion in contact with the stack 2, it is possible to prevent heat transfer from the workpieces constituting the stack 2 to the jig 4, and thus it is possible to prevent the workpieces on the lower portion and/or the upper portion of the stack 2 from having a lower temperature than the other workpieces. A pressing force of the pressing portion 15 is applied to the heat insulating member. Therefore, a material constituting the heat insulating member preferably has resistance against such pressing force. Examples of such material include a carbon plate material, an electrically insulating heat insulating plate such as NEOARK (Japan registered trademark No. 4246196), and a calcium silicate heat insulating plate made such as LUMIBOARD (Japan trademark application No. 2020-071159).

In the above embodiment, the jig 4 includes the accommodation portion 7, and the jig 4 moves in the transport path 5 together with the accommodation portion 7 so as to be heated from the outside of the accommodation portion 7 by the heating apparatus 6, whereas the friction material manufacturing apparatus 1 may be configured such that the accommodation portion 7 collectively accommodates the jig 4, the transport path 5, and the heating apparatus 6, or alternatively, the accommodation portion 7 accommodates the heating apparatus 6 and the jig 4 can move in and out from the accommodation portion 7.

Fig. 9 is a diagram showing a first modification of the friction material manufacturing apparatus 1. In the friction material manufacturing apparatus 1 of the above embodiment, for example, as shown in Fig. 9, the accommodation portion 7 may be configured to collectively accommodate the jig 4, the transport path 5, and the heating apparatus 6. In the present modification, since the heating apparatus 6 is accommodated in the accommodation portion 7, the quartz glass 13 is not necessary. Therefore, supply of a gas for preventing contamination of the quartz glass 13 is not necessary, and a gas for discharging vaporized components vaporized from the workpieces due to heating is supplied into the accommodation portion 7. In this case, it is preferable that the accommodation portion 7 is provided with a door that allows the workpieces to be attached to the jig 4 or allows the jig 4 to move.

In the friction material manufacturing apparatus 1 of this modified example, it is not necessary to connect the jig 4 to the inert gas cylinder 10 by the hose 11. Therefore, the jig 4 can be easily handled. Fig. 10 is a structural view of the friction material manufacturing apparatus according to the first modification as viewed from a lateral side of the transport path. As shown in Fig. 10, the inert gas cylinder 10 is connected by a hose to the gas introduction portion of the accommodation portion 7 that collectively accommodates the jig 4, the transport path 5, and the heating apparatus 6. The jig 4 is accommodated in the accommodation portion 7, and is not connected to the inert gas cylinder 10. Therefore, in the friction material manufacturing apparatus 1 according to the present modification, when the jig 4 is moved along the transport path 5, the hose connected to the inert gas cylinder 10 does not hinder movement of the jig 4. Therefore, the jig 4 can be easily moved along the transport path 5.

Fig. 11 is a diagram showing a second modification of the friction material manufacturing apparatus 1. The friction material manufacturing apparatus 1 of the above embodiment may be such that, for example, as shown in Fig. 11, the accommodation portion 7 is provided in the heating apparatus 6, and the jig 4 before heating and the jig 4 after heating are disposed outside the accommodation portion 7. In this case, an opening that allows the jig 4 to move in and out, and a door for opening and closing the opening are provided on both side surfaces of the accommodation portion 7. When the opening is closed by the door to close the accommodation portion, the inside of the accommodation portion can be filled with the gas supplied from the inert gas cylinder 10. In this modification, similarly to the first modification, since the heating apparatus 6 is accommodated in the accommodation portion 7, the quartz glass 13 is not necessary.

Fig. 12 is a diagram showing a third modification of the friction material manufacturing apparatus 1. The friction material manufacturing apparatus 1 of the above embodiment may be such that, for example, as shown in Fig. 12, the jig 4 before heating and the heating apparatus 6 are accommodated in the accommodation portion 7, and the jig 4 after heating is disposed outside the accommodation portion 7. In this case, an opening that allows the jig 4 to move in and out, and a door for opening and closing the opening are provided on a side surface of the accommodation portion 7. When the opening is closed by the door to close the accommodation portion, the inside of the accommodation portion can be filled with the gas supplied from the inert gas cylinder 10. In this modification, similarly to the first modification and the second modification, since the heating apparatus 6 is accommodated in the accommodation portion 7, the quartz glass 13 is not necessary.

Fig. 13 is a diagram showing a fourth modification of the friction material manufacturing apparatus 1. The friction material manufacturing apparatus 1 of the above embodiment may be such that, for example, as shown in Fig. 13, the jig 4 after heating and the heating apparatus 6 are accommodated in the accommodation portion 7, and the jig 4 before heating is disposed outside the accommodation portion 7. In this case, an opening that allows the jig 4 to move in and out, and a door for opening and closing the opening are provided on a side surface of the accommodation portion 7. When the opening is closed by the door to close the accommodation portion, the inside of the accommodation portion can be filled with the gas supplied from the inert gas cylinder 10. In this modification, similarly to the first modification, the second modification, and the third modification, since the heating apparatus 6 is accommodated in the accommodation portion 7, the quartz glass 13 is not necessary.

### REFERENCE SIGNS LIST

- 1: friction material manufacturing apparatus
- 2: stack
- 3: pressing mechanism
- 4: jig
- 5: transport path
- 6: heating apparatus
- 7: accommodation portion
- 8: transport mechanism
- 9: support member
- 10: inert gas cylinder
- 11: hose
- 12: gas introduction port
- 13: quartz glass
- 14: support portion
- 15: pressing portion
- 16: air cylinder
- 17: gas exhaust port

## Claims

1. A friction material manufacturing apparatus (1) for sintering friction materials, the friction material manufacturing apparatus (1) comprising:
a jig (4) configured to clamp a stack (2) of workpieces, which are preforms of the friction materials, in a stacking direction;
a transport mechanism (8) that forms a transport path (5) of the jig (4); and
a heating apparatus (6) provided in a way of the transport path (5) and configured to heat the stack clamped by the jig (4) with infrared rays from a lateral side with respect to the stacking direction.

2. The friction material manufacturing apparatus (1) according to claim 1,
wherein the jig (4) includes:
a support portion (14) configured to support the stack (2) from one side in the stacking direction; and
a pressing portion (15) configured to press the stack (2) from the other side in the stacking direction toward the support portion (14).

3. The friction material manufacturing apparatus (1) according to claim 1 or 2,
wherein the heating apparatus (6) includes an element configured to emit infrared rays and disposed at a position that is on the lateral side of the stack (2) in a state where the jig (4) is at a position of the heating apparatus (6).

4. The friction material manufacturing apparatus (1) according to claim any one of claims 1 to 3, wherein
the jig (4) includes an accommodation portion (7) configured to accommodate the stack (2), and
the accommodation portion (7) includes a window (13) made from a transparent plate configured to cover the stack (2) from the lateral side with respect to the stacking direction.

5. The friction material manufacturing apparatus (1) according to claim 4,
wherein the jig (4) includes a gas introduction portion (12) configured to introduce an inert gas into the accommodation portion (7).

6. The friction material manufacturing apparatus (1) according to claim any one of claims 1 to 3, further comprising:
an accommodation portion (7) configured to accommodate the jig (4), the transport mechanism (8), and the heating apparatus (6).

7. The friction material manufacturing apparatus (1) according to claim any one of claims 1 to 3, further comprising:
an accommodation portion (7) configured to accommodate the heating apparatus (6), and allow the jig (4) to move in and out.

8. The friction material manufacturing apparatus (1) according to claim 7,
wherein the accommodation portion (1) includes a door at an opening portion through which the jig (4) is to move in and out.

9. The friction material manufacturing apparatus (1) according to claim any one of claims 6 to 8,
wherein the accommodation portion (7) includes a gas introduction portion (12) configured to introduce an inert gas.

10. The friction material manufacturing apparatus (1) according to claim any one of claims 1 to 9,
wherein the jig (4) includes a heat insulating member at a portion to be in contact with the stack (2).

11. The friction material manufacturing apparatus (1) according to claim any one of claims 1 to 10,
wherein the heating apparatus (6) is a near infrared heater having a peak wavelength in a range of 1200 nm to 1700 nm.

12. A friction material manufacturing method for sintering friction materials, the friction material manufacturing method comprising:
clamping, by a jig (4), a stack (2) of workpieces, which are preforms of the friction materials, in a stacking direction;
transporting the jig (4) along a transport path (5) formed by a transport mechanism (8); and
heating, by a heating apparatus (6) provided in a way of the transport path (5), the stack (2) clamped by the jig (4) with infrared rays from a lateral side with respect to the stacking direction.

## Patentansprüche

1. Vorrichtung (1) zur Herstellung von Reibmaterialien zum Sintern von Reibmaterialien, wobei die Vorrichtung (1) zur Herstellung von Reibmaterialien umfasst:
eine Spannvorrichtung (4), die so konfiguriert ist, dass sie einen Stapel (2) von Werkstücken, die Vorformen der Reibmaterialien sind, in einer Stapelrichtung einspannt;
einen Transportmechanismus (8), der einen Transportweg (5) der Spannvorrichtung (4) bildet; und
eine Heizvorrichtung (6), die in einem Weg des Transportweges (5) vorgesehen und so konfiguriert ist, dass sie den von der Spannvorrichtung (4) eingespannten Stapel mit Infrarotstrahlen von einer seitlichen Seite in Bezug auf die Stapelrichtung erwärmt.

2. Vorrichtung (1) zur Herstellung von Reibmaterial nach Anspruch 1,
wobei die Spannvorrichtung (4) umfasst:
einen Stützabschnitt (14), der so konfiguriert ist, dass er den Stapel (2) von einer Seite in der Stapelrichtung stützt; und
einen Pressabschnitt (15), der so konfiguriert ist, dass er den Stapel (2) von der anderen Seite in der Stapelrichtung gegen den Stützabschnitt (14) drückt.

3. Vorrichtung (1) zur Herstellung von Reibmaterial nach Anspruch 1 oder 2,
wobei die Heizvorrichtung (6) ein Element enthält, das so konfiguriert ist, dass es Infrarotstrahlen emittiert, und das an einer Position angeordnet ist, die sich an der Seite des Stapels (2) in einem Zustand befindet, in dem sich die Spannvorrichtung (4) an einer Position der Heizvorrichtung (6) befindet.

4. Vorrichtung (1) zur Herstellung von Reibmaterial nach einem der Ansprüche 1 bis 3, wobei
die Spannvorrichtung (4) einen Aufnahmeabschnitt (7) aufweist, der zur Aufnahme des Stapels (2) konfiguriert ist, und
der Aufnahmeabschnitt (7) ein Fenster (13) aufweist, das aus einer transparenten Platte hergestellt ist, die so konfiguriert ist, dass sie den Stapel (2) von der seitlichen Seite in Bezug auf die Stapelrichtung abdeckt.

5. Vorrichtung (1) zur Herstellung von Reibmaterial nach Anspruch 4,
wobei die Spannvorrichtung (4) einen Gaseinführungsabschnitt (12) aufweist, der so konfiguriert ist, dass er ein Inertgas in den Aufnahmeabschnitt (7) einführt.

6. Vorrichtung (1) zur Herstellung von Reibmaterial nach einem der Ansprüche 1 bis 3, ferner umfassend:
einen Aufnahmeabschnitt (7), der so gestaltet ist, dass er die Spannvorrichtung (4), den Transportmechanismus (8) und die Heizvorrichtung (6) aufnimmt.

7. Vorrichtung (1) zur Herstellung von Reibmaterial nach einem der Ansprüche 1 bis 3, ferner umfassend:
einen Aufnahmeabschnitt (7), der so konfiguriert ist, dass er die Heizvorrichtung (6) aufnimmt und das Ein- und Ausfahren der Spannvorrichtung (4) ermöglicht.

8. Vorrichtung (1) zur Herstellung von Reibmaterial nach Anspruch 7,
wobei der Aufnahmeabschnitt tt (1) eine Tür an einem Öffnungsabschnitt aufweist, durch den die Spannvorrichtung (4) hinein- und herausbewegt werden soll.

9. Vorrichtung (1) zur Herstellung von Reibmaterial nach einem der Ansprüche 6 bis 8,
wobei der Aufnahmeabschnitt (7) einen Gaseinführungsabschnitt (12) aufweist, der zum Einführen eines Inertgases konfiguriert ist.

10. Vorrichtung (1) zur Herstellung von Reibmaterial nach einem der Ansprüche 1 bis 9,
wobei die Spannvorrichtung (4) ein wärmeisolierendes Element an einem Abschnitt aufweist, der mit dem Stapel (2) in Kontakt steht.

11. Vorrichtung (1) zur Herstellung von Reibmaterial nach einem der Ansprüche 1 bis 10,
wobei die Heizvorrichtung (6) ein Nahinfrarotstrahler mit einer Spitzenwellenlänge im Bereich von 1200 nm bis 1700 nm ist.

12. Verfahren zur Herstellung von Reibwerkstoffen zum Sintern von Reibwerkstoffen, wobei das Verfahren zur Herstellung von Reibwerkstoffen Folgendes umfasst:
Einspannen eines Stapels (2) von Werkstücken, bei denen es sich um Vorformlinge der Reibmaterialien handelt, in einer Stapelrichtung mittels einer Spannvorrichtung (4);
Transportieren der Spannvorrichtung (4) entlang eines Transportweges (5), der durch einen Transportmechanismus (8) gebildet wird; und
Erwärmen des von der Spannvorrichtung (4) eingespannten Stapels (2) mit Infrarotstrahlen von einer Seite in Bezug auf die Stapelrichtung durch eine Heizvorrichtung (6), die in einem Weg des Transportweges (5) vorgesehen ist.

## Revendications

1. Dispositif de production de matériau de friction (1) pour le frittage de matériau de friction, le dispositif de production de matériau de friction (1) comprenant :
un gabarit (4) configuré pour serrer une pile (2) de pièces, qui sont des préformes des matériaux de friction, dans une direction d'empilage ;
un mécanisme de transport (8) qui forme un chemin de transport (5) du gabarit (4) ; et
un dispositif de chauffage (6) placé sur le chemin de transport (5) et configuré pour chauffer la pile serrée par le gabarit (4) à l'aide de rayons infrarouges depuis un côté latéral par rapport à la direction d'empilage.

2. Dispositif de production de matériau de friction (1) selon la revendication 1,
dans lequel le gabarit (4) comprend :
une partie de support (14) configurée pour soutenir la pile (2) d'un côté dans la direction d'empilage ; et
une partie de pressage (15) configurée pour presser la pile (2) de l'autre côté dans la direction d'empilage vers la partie de support (14).

3. Dispositif de production de matériau de friction (1) selon les revendications 1 ou 2,
dans lequel le dispositif de chauffage (6) comprend un élément configuré pour émettre des rayons infrarouges et disposé à une position qui est sur le côté latéral de la pile (2) dans un état où le gabarit (4) est à une position du dispositif de chauffage (6).

4. Dispositif de production de matériau de friction (1) selon l'une des revendications 1 à 3, dans lequel
le gabarit (4) comprend une partie de logement (7) configurée pour accueillir la pile (2), et
la partie d'accueil (7) comprend une fenêtre (13) fabriquée à partir d'une plaque transparente configurée pour couvrir la pile (2) du côté latéral par rapport à la direction d'empilage.

5. Dispositif de production de matériau de friction (1) selon la revendication 4,
dans lequel le gabarit (4) comprend une partie d'introduction de gaz (12) configurée pour introduire un gaz inerte dans la partie hébergement (7).

6. Dispositif de production de matériau de friction (1) selon l'une des revendications 1 à 3, comprenant en outre :
une partie hébergement (7) configurée pour accueillir le gabarit (4), le mécanisme de transport (8) et le dispositif de chauffage (6).

7. Dispositif de production de matériau de friction (1) selon l'une quelconque des revendications 1 à 3, comprenant en outre :
une partie hébergement (7) configurée pour accueillir le dispositif de chauffage (6), et permettre au gabarit (4) de se déplacer à l'intérieur et à l'extérieur.

8. Dispositif de production de matériau de friction (1) selon la revendication 7,
dans lequel la partie hébergement (1) comprend une porte au niveau d'une partie ouverture à travers laquelle le gabarit (4) doit entrer et sortir.

9. Dispositif de production de matériau de friction (1) selon l'une des revendications 6 à 8, dans lequel la partie hébergement (7) comprend une partie d'introduction de gaz (12) configurée pour introduire un gaz inerte.

10. Dispositif de production de matériau de friction (1) selon l'une quelconque des revendications 1 à 9,
dans lequel le gabarit (4) comprend un élément d'isolation thermique au niveau d'une partie destinée à être en contact avec la pile (2).

11. Dispositif de production de matériau de friction (1) selon l'une quelconque des revendications 1 à 10,
dans lequel le dispositif de chauffage (6) est un dispositif de chauffage proche infrarouge dont la longueur d'onde de crête se situe dans une plage de 1200 nm à 1700 nm.

12. Production de production de matériau de friction par frittage, le procédé de production de matériau de friction comprenant :
le serrage, par un gabarit (4), d'une pile (2) de pièces, qui sont des préformes des matériaux de friction, dans une direction d'empilage ;
le transport du gabarit (4) le long d'un chemin de transport (5) formé par un mécanisme de transport (8) ; et
le chauffage, à l'aide d'un dispositif de chauffage (6) placé sur le chemin de transport (5), de la pile (2) serrée par le gabarit (4) à l'aide de rayons infrarouges depuis un côté latéral par rapport à la direction de l'empilage.
